

April 30, 1957

R. H. SONNEBORN ET AL

2,790,741

BONDED FIBROUS PRODUCTS AND METHOD OF MANUFACTURE

Filed Sept. 30, 1952

FIG-1a



FIG-1b



INVENTORS  
RALPH H. SONNEBORN  
THOMAS E. PHILIPPS  
BY

*Stahl & Oberman*  
ATTYS

1

2,790,741

**BONDED FIBROUS PRODUCTS AND METHOD OF MANUFACTURE**

Ralph H. Sonneborn, Newark, and Thomas E. Philipp, Granville, Ohio, assignors to Owens-Corning Fiberglas Corporation, Toledo, Ohio, a corporation of Delaware

Application September 30, 1952, Serial No. 312,198

8 Claims. (Cl. 154—101)

This invention relates to methods and apparatus for making fibrous products and especially to methods of applying binders to such products.

In the past, various resinous products including resins in the form of granular powders and liquid resins have been applied to fibrous glass products as binding material to give the finished products integrity and strength. Formerly, such liquid resins or granular powder resins have been applied in various ways including the use of spraying and dusting methods; however, the problem of obtaining the proper distribution of binding material throughout the product has always been present and not too successfully met by the former methods.

One of the methods used formerly in applying binder was to spray a water dispersion of the resinous material upon the fibrous glass as the fibers themselves were being formed. This method results in a product having fairly uniform binder distribution and good strength of product. However, this method makes it necessary to drive off in subsequent heating operations a great deal of water or solvent dependent upon which medium is present. The heating step requires much time and the use of a great deal of energy.

Another method formerly used has been to form a mat of fibers upon which is dusted a powdered resinous material which can be set by application of heat to the mat. The products so formed tend to have a weak or low tensile strength and high ignition losses which indicates that the proportion of binder ingredient is too high without actually giving adequate strength in the product itself. The low strength results at least partially because of the non-uniform distribution of the binder throughout the mat.

It is an object of this invention to obtain uniform distribution of binder materials in fibrous mats and the like.

It is also an object to provide a method of producing uniformly bonded mats of any thickness, including very thick mats.

It is a further object to provide a continuous method of producing mats having good integrity and high tensile strength.

It is an object to provide a method of reducing the binder-to-fiber ratio while improving the quality of the final product.

Other objects will be evident from the description and drawings in which:

Figures 1a and 1b constitute a schematic view of apparatus with which this invention may be carried out; and

Figure 2 is an enlarged view of the product showing the fused powdered binder on the inner fibers of the layer of mat and heatset sprayed resinous binder on the outer layers of the mat.

This apparatus is used to apply first a powdered resinous binder and then a sprayable liquid binder in such a manner that, although reduced proportions of binder are used, a better product is obtained because the uniformity of distribution of the binder is improved and

2

resulting higher strengths of the product are attained. The combination of the application of powdered and liquid binders to a fibrous mat and especially the application of the powdered and liquid binders in the sequence used in this invention is believed to be new in the art and entirely unobvious for it is a radical departure from the sequence generally used in applying liquid and powdered materials on the same product. Normally, it would seem best to apply first the liquid and then the powder; however, it has been discovered that the best results are attained by applying the binder materials in the reverse of the obvious order as will be described in the following paragraphs. Furthermore it has been discovered that the total binder content can be lowered even though two forms of binder are applied to the product.

In Figure 1A, the apparatus comprises a cutter 12, into which a plurality of strands 11 of fibrous glass are being fed. The cutter 12 comprises a pair of opposed rolls 13 and 14, the former being a rubber-covered roll and the latter being provided with cutterbars 15, 15 arranged longitudinally across the periphery of the roll. Roll 13 is driven by a suitable mechanism indicated by numeral 16. Roll 14 is in turn driven through the gear train including gears 17 and 18.

A conveyor belt 19, mounted on rolls 21 and 22, lies generally below the cutter 12. Conveyor belt 19 is a mesh belt and is provided with a suction box 23 having a vacuum line 24. Chopped strands 25, 25 are retained by members 26, 26. An inclined conveyor belt 27, mounted on rolls 28 and 29, is situated adjacent to conveyor belt 19 with rolls 22 and 28 being immediately adjacent one another. The mat of fibrous material 31 is shown on both conveyor belts 19 and 27.

Above conveyor belt 27 and near roll 29 is mounted a hopper 32 containing a suitable powdered binder 33. Immediately adjacent roll 29 is a picker roll 34 having tooth-like prongs 35, 35. Between retaining members 36 and 37 is shown a mixture of powdered binder and chopped fibrous material 38. This mixture 38 is shown being deposited on conveyor belt 39 which is mounted upon rolls 41 and 42. Conveyor belt 39 is provided with a suction box 30 having vacuum line 40.

Conveyor belt 39 and roll 42 appear in Figure 1B where a mat of chopped fibrous material and powdered binder 43 is shown passing over conveyor belt 39 after being formed thereon. Disposed above conveyor belt 39 is a bank of spray nozzles 44, 44 mounted upon manifold 45 to which is supplied a suitable liquid resinous binder. Next to conveyor belt 39 is another conveyor belt 46 which is mounted upon rolls 47, 48. Between rolls 42 and 47 is mounted a bank of nozzles 49, 49 mounted upon manifold 51 which manifold is supplied with a liquid resinous binder shown being sprayed upon the mat 43.

Belts 19 and 39 are mesh belts through which air can pass while belt 46 is preferably one which can withstand high temperatures but need not necessarily be one through which air can pass. About conveyor belt 46 is oven 52 heated by any suitable heat source and designed to fuse and heat set the binders which have been applied to the mat product. The final product 53 is rolled up by means not shown.

In using this apparatus, the strands 11 are pulled from a creel, not shown, containing packages of the strand and are threaded between idler roll 10 and rubber covered roll 13. The cutter 12 is then started so that the strands 11, 11 are pulled between rolls 13 and 14 and are chopped into lengths of from  $\frac{1}{2}$  to 5 inches as may be desired. The chopped strands then fall, due to gravity, upon conveyor belt 19 and are pulled downwardly upon the belt by the action of suction box 23. The retain-

ing members 26, 26 confine the chopped strands as they are falling from the cutter 12, and after the chopped strands are pulled downwardly into a mat upon conveyor belt 19, they move toward conveyor belt 27 and proceed upwardly upon this belt as can be seen in Figure 1A. A powdered resinous material comprising a phenol formaldehyde resin is then applied through the bottom of hopper 32 and the powdered binder passes downwardly throughout the extent of the mat of fibrous material. The mat then passes into a picker roll 34 which very intimately mixes powdered binder and short chopped strands of fibrous material. The picker roll also destroys the integrity of the mat 31, resulting in the deposition of a mixture of fibrous material and powdered binder upon conveyor belt 39 in that area between retaining members 36 and 37. The mat of chopped fiber and powdered binder 43 is then formed by the action of suction box 30 and this mat passes over conveyor belt 39 and is sprayed both on top and bottom by nozzles 45, 45 and 49, 49. A liquid resinous binder comprising a water dispersion of phenol formaldehyde resin is used to coat the upper and lower surfaces of the mat. The mat proceeds over conveyor belt 46 through the heated oven 52 wherein the powdered binder is fused and the liquid binder which covers the upper and lower surfaces of the mat is heat set and becomes an integral part of the final product.

In Figure 2 a view of the final product greatly enlarged is shown. The inner fibers 54 of this product are bonded one to another chiefly by spherical particles of binder formed by fusing the powdered binder which has been applied. The upper and lower surfaces 55 of the product are bonded one to another mainly by a thin coating of resin formed from a liquid film applied by spray nozzles 45, 45 and 49, 49.

Various binders may be used; both powdered and liquid binders may be chosen for their particular desirable properties. For instance, phenol formaldehyde, urea formaldehyde, polyvinyl acetate, melamine and polystyrene resins, polyester resins such as those formed from the reaction of diethylene glycol and maleic anhydride cross-linked with diallyl phthalate, resins formed from a polyol and fumaric acid, and others may be used. Any resin which may be heat treated to form a binder for the fibrous material may be used. It is intended, however, to use a combination of a dry particulate binder material along with a liquid binder material, which liquid may be either in the form of a solution in a solvent system or an emulsion or dispersion in either a compatible liquid or a water system.

Oven temperatures may vary according to the particular resins used. However, the temperatures will generally vary from about 180° F. to about 700° F. and possibly as high as 1000° F.

The percent of solids in the liquid binder may be varied as may be necessary in forming handleable emulsions or dispersions of the different resins which are used. The emulsions or dispersions may vary from 1/4 to 40% total solids dependent upon the resin used. Low percentage emulsions of polyester type resins may be used, for instance, if a diallyl phthalate polyester copolymer is used, a 2% emulsion may be used.

The percent of binder in the finished product may vary considerably; however, the total weight of binder will generally vary from about 4 to 15% resin. Half of this binder percentage may be powdered resin and half liquid resin; however, it is obvious that this 50-50 ratio need not be maintained. For instance, a greater percentage of the final resin content may result from addition of powdered binder. In fact, 90 or more percent of the final resin content may be due to either the powdered or the liquid resin. Preferably the total binder percentage will comprise 40 to 60% binder added as a powder and 60 to 40% binder added as an emulsion or dispersion.

It has been discovered that great savings can be realized by adding the resinous binder in two forms, namely, a powder form and a liquid form. Furthermore, it has been discovered that by adding the powdered binder first, it is possible to get complete uniformity of binder distribution within the mat since it is believed the powdered binder drops downwardly throughout the mat when it is applied and then subsequently the liquid binder coats the surfaces and the interstices of the mat to produce a mat having great integrity and tensile strength. To add the liquid and powdered binders in another sequence would result in all or a greater proportion of the binder being deposited upon the surface of the mat and would result in a weak and non-uniform product.

Although in the example illustrated by the drawings, the powdered binder and fibers of the mat 31 are intimately mixed by disrupting the mat integrity, it should be understood that violent action need not be taken. The mat as first formed can remain intact throughout the treatment and the powdered binder can be distributed throughout the mat by shaking the mat.

The methods and apparatus of this invention can be used to produce mats of any fibrous material including hair, straw glass, felt, cellulose, silk, wool, and any 25 of the synthetic fibers, including those comprising a polyamide, a polymer of vinyl chloride and acrylonitrile, polyacrylonitrile, a polymer of ethylene glycol and dimethyl terephthalate, a polymer of vinylidene chloride and vinyl chloride, and others.

Although a particular embodiment of the invention has been disclosed, obvious modifications may be made within the spirit and scope of the following claims.

We claim:

1. A method of producing a resin bonded fibrous glass mat comprising chopping and collecting fibrous glass material in the form of an advancing mat, distributing on said advancing mat a powdered heat setting resinous binder, mechanically disrupting the fibrous glass material within said advancing mat to form an intimate mixture of said fibrous glass material and said powdered resinous binder, collecting said mixture in the form of an advancing mat, spraying a heat setting, resinous binder in liquid form upon the advancing mat, and subjecting said mat to an elevated temperature to heat set the resinous binders thereon.

2. An integral mat of haphazardly arranged fibers of glass bonded together by a resinous binder, the inner fibers of said mat being bonded one to another chiefly by fused particles of a dry resinous binder, and the 50 outer fibers of which are bonded one to another by a uniform coating of resinous binder material, the binders being selected from the group of resins consisting of phenol formaldehyde, urea formaldehyde, polyvinyl acetate, melamine, polystyrene, and polyesters.

3. The mat of claim 2 wherein said fused particles of dry resinous binder comprise from 40 to 60 parts by weight of the total weight of the resinous binder, and said uniform coating of resinous binder comprises from 40 to 60 parts by weight of the total weight of resinous binder, said resinous binder being from 4 to 15 percent by weight of the mat.

4. A mat of haphazardly arranged chopped textile strands of glass bonded with a phenol formaldehyde binder, the chopped textile strands of the body of said 65 mat being bonded one to another chiefly by fused particles of dry phenol formaldehyde binder, the chopped textile strands at the surfaces of said mat being bonded one to another by a thin coating of phenol formaldehyde resin binder, said fused particles of a dry phenol formaldehyde 70 binder comprising from 40 to 60 percent of the total weight of binder and said thin coating of resinous binder comprising from 40 to 60 percent of the total weight of binder, the total binder content being from 4 to 15 percent by weight.

5. A mat of haphazardly arranged chopped textile

strands of glass bonded with a heat setting resin, the chopped textile strands of the body of said mat being bonded one to another by particles of a polyester resin applied as a powder, the chopped textile strands at the surface of said mat being bonded one to another by a coating of polyester resin applied as a liquid, said particles of resin applied as a powder comprising from 40 to 60 parts by weight of the total weight of the resin and said coating of resin applied as a liquid comprising from 40 to 60 parts by weight of the total weight of resin, the total resin content being from 4 to 15 percent by weight of the mat.

6. The mat of claim 5 wherein the polyester resin is one produced by the reaction of diethylene glycol and maleic anhydride cross-linked with diallyl phthalate.

7. A method of producing a resin bonded fibrous glass mat comprising chopping and collecting fibrous glass strands to form an advancing mat, introducing into said advancing mat a powdered resin selected from the group consisting of phenol formaldehyde, urea formaldehyde, polyvinyl acetate, melamine, polystyrene and polyester resins, intimately mixing said fibrous glass strands and said powdered resin in said advancing mat, applying to at least one surface of said advancing mat a liquid resin selected from the group consisting of phenol formaldehyde, urea formaldehyde, polyvinyl acetate, melamine, polystyrene and polyester resins, and heating said mat to set the powdered and liquid resins, the powdered and liquid resins each being introduced in sufficient quantity to provide from 40 to 60 percent of the total binder content, said binder being from 4 to 15 percent by weight of the mat.

8. In a continuous method of producing resin bonded fibrous glass mat comprising cutting and collecting fibrous

glass strands in the form of an advancing mat, the steps comprising applying a dry powdered polyester resin to said advancing mat, mechanically disrupting the integrity of said advancing mat and forming an intimate mixture of said fibrous glass strands of said advancing mat with said dry powdered polyester resin, collecting said intimate mixture in the form of a secondary advancing mat, applying a liquid polyester resin in the form of an emulsion to the surface of said secondary advancing mat, and heating to set both the dry powdered polyester resin and the liquid polyester resin, the powdered and liquid resins each being introduced in sufficient quantity to provide from 40 to 60 percent of the total resin content, the total resin content being from 4 to 15 percent by weight of the mat.

#### References Cited in the file of this patent

#### UNITED STATES PATENTS

|           |                    |                |
|-----------|--------------------|----------------|
| 1,880,930 | Elbel et al. ----- | Oct. 4, 1932   |
| 1,928,264 | Powell -----       | Sept. 26, 1933 |
| 1,952,208 | Hussey -----       | Mar. 27, 1934  |
| 2,057,166 | Schur -----        | Oct. 13, 1936  |
| 2,288,072 | Collins -----      | June 30, 1942  |
| 2,292,118 | Guhl -----         | Aug. 4, 1942   |
| 2,372,433 | Koon -----         | May 27, 1945   |
| 2,373,033 | Kopplin -----      | Apr. 3, 1945   |
| 2,566,960 | Philipps -----     | Sept. 4, 1951  |
| 2,569,169 | Heritage -----     | Sept. 25, 1951 |
| 2,579,770 | Uschmann -----     | Dec. 25, 1951  |
| 2,619,151 | Sheidley -----     | Nov. 25, 1952  |
| 2,698,271 | Clark -----        | Dec. 28, 1954  |

#### FOREIGN PATENTS

Great Britain ----- Mar. 12, 1952